

## UNITED STATES PATENT OFFICE

2,400,905

EXPANSION CONTROL OF MOLDS AND  
THE LIKE

Xarifa L. Bean, Yellow Springs, Ohio, assignor to  
Antioch College, a corporation of Ohio, Morris  
Bean, Xarifa Bean, Algo D. Henderson, Arthur  
E. Morgan, and William Beatty, all of Yellow  
Springs, Ohio

No Drawing. Application October 15, 1943,  
Serial No. 506,425

10 Claims. (Cl. 22—188)

This invention relates generally to molds for use in metal casting and more particularly to expansion control agents for use in plaster molds in which the molten metal is to be poured in the casting process.

In the manufacture of non-ferrous metal castings, particularly aluminum and aluminum alloy castings in plaster of Paris bonded molds, one of the difficulties encountered with addition agents heretofore employed to control the processing expansion of molds is that these addition agents have sometimes caused an objectionable efflorescence or blooming of the mold surface. Serious surface buckling may also result. To overcome these difficulties requires expensive processing and constant inspection and retouching.

The problem has been encountered in the manufacture of aluminum alloy castings in molds according to the process of Bean Patent 2,220,703 granted November 5, 1940. According to the Bean process, after the initial set the mold is placed in an autoclave, and subjected to steam under pressure to convert calcium sulfate di-hydrate to calcium sulfate hemi-hydrate and to leave free water distributed throughout the plaster. The mold is thereafter removed from the autoclave and allowed to stand for a number of hours at room temperature whereby the hemi-hydrate is rehydrated to di-hydrate. The mold thereafter is dried to remove free water from the plaster. The effect of this treatment is to increase the permeability of the material so as to permit escape of gases generated in the mold during casting while providing a smooth skin at the surface of the mold giving better definition to the surface of the casting.

The problem of selecting suitable expansion control agents for plaster bonded molds is complicated and has to take into consideration a number of factors. In addition to controlling satisfactorily both the initial setting and processing expansion (brought about by the pressure vessel dehydrating and room rehydrating of the Bean process), consideration must be given to the effect of the control agent on other major properties and attributes of the mold material, such as setting time, green strength, processing time, surface quality, dry strength, permeability and heat absorption rate. For example some expansion control agents are powerful accelerators, causing the plaster to set almost instantly. Others are powerful retarders or inhibitors. Some agents will cause the green strength to be but a fraction of what it would be otherwise.

Some have an adverse effect on the permeability of the finished mold.

I have discovered as a result of considerable work and experimentation that sodium aluminate or potassium aluminate added in small amounts, controls both the expansion due to the initial setting of the plaster and that due to autoclave dehydrating and subsequent rehydrating steps of the Bean process and that these aluminates otherwise successfully meet the requirements of a suitable control agent as outlined.

The sodium or potassium aluminate in powdered form is added to and thoroughly mixed with the dry plaster of Paris and the other components of the dry plaster mix. A small amount of control agent is all that is required. Very satisfactory results have been obtained with an addition of from 4% to 1% by weight of the sodium or potassium aluminate.

20 After the dry mixture including the control agent has been thus prepared, water is added thereto to form a wet mix from which the mold is formed. After the wet plaster forming the mold has set, the mold is processed with steam under pressure in an autoclave to convert the calcium sulfate di-hydrate to calcium sulfate hemi-hydrate and to leave free water distributed throughout the mold. The mold is removed from the autoclave and allowed to stand at room temperature for a number of hours whereby the hemi-hydrate is rehydrated to di-hydrate. The mold is then dried to remove practically all of the remaining free water from the plaster.

25 In addition to being an effective expansion control agent, the sodium or potassium aluminate is an inhibitor of "mold reaction". Mold reaction causes a kind of porosity in the metal castings being produced, the amount of which can be determined by X-ray analysis of the castings.

30 It appears that the condition may be caused by gases formed by reaction between one or more of the components of the mold and one or more components of the molten metal or alloy being cast in the mold. An illustrative example of an aluminum alloy which reacts with molds containing calcium sulfate is one composed of 5% silicon, 1.3% copper, 0.5% magnesium, balance aluminum plus traces of impurities normally present in aluminum alloys. Sodium aluminate or potassium aluminate is an effective inhibitor of mold reaction such as that encountered with the above described aluminum alloy.

35 While the specific embodiment of the invention described herein deals with expansion control agents for molds, it will be understood that

the principles of the invention have application in the making of cores in which expansion is to be controlled.

Various changes and modifications of the embodiment of my invention described herein may be made without departing from the principle and spirit of the invention.

I claim:

1. The method of controlling expansion in a plaster of Paris mold or core which includes adding an alkali metal aluminate to the dry plaster mix.

2. The method of controlling expansion in a plaster of Paris bonded mold or core which includes adding a small amount of an alkali metal aluminate to the dry mix.

3. A plaster of Paris mold containing a small amount of an alkali metal aluminate.

4. The method of forming a plaster of Paris mold which includes forming a desired mold shape from a mixture comprising plaster of Paris, a small amount of an alkali metal aluminate and

water, setting the plaster, dehydrating the set plaster to convert calcium sulfate di-hydrate to calcium sulfate hemi-hydrate and to leave free water distributed throughout the mold, thereafter rehydrating the hemi-hydrate to di-hydrate and then drying the mold to remove practically all of the remaining free water from the plaster.

5. A mold as in claim 3 in which the aluminate is sodium aluminate.

6. A mold as in claim 3 in which the aluminate is potassium aluminate.

7. The method as in claim 4 in which the aluminate is sodium aluminate.

8. The method as in claim 4 in which the aluminate is potassium aluminate.

9. A mold as in claim 3 in which about .4% to 1% by weight of sodium aluminate is present in the mold.

10. The method as in claim 4 in which about .4% to 1% by weight of sodium aluminate is employed.

XARIFA L. BEAN.